

# United States Patent Office

2,841,512

Patented July 1, 1958

1

2,841,512

## METHOD OF WORKING AND HEAT TREATING ALUMINUM-MAGNESIUM ALLOYS AND PRODUCT THEREOF

Hugh S. Cooper, Shaker Heights, Ohio, assignor to William F. Jobbins, Incorporated, Aurora, Ill., a corporation of Illinois

No Drawing. Application October 12, 1956  
Serial No. 615,456

8 Claims. (Cl. 148—11.5)

This invention relates to aluminum alloys in which magnesium is a major alloying element and it relates more particularly to the provision of aluminum-magnesium alloys which are wrought alloys, having been fabricated by forging, rolling, extruding and other fabricating procedures involving substantial mechanical working.

Wrought alloys which are known as heat-treatable alloys comprise those in which solid solution and precipitation heat treatments produce the desired tempers in the final product, while non-heat-treatable wrought alloys comprise those where the various tempers are produced by strain hardening or the like, solution heat treatment having no significant effect. While the former have generally highest strengths, they are characterized by low corrosion resistance, particularly in the case of aluminum-magnesium heat-treatable alloys (this low resistance apparently involves predominantly the phenomenon known as "stress corrosion"). These heat-treatable alloys must therefore be protected by cladding in many if not most applications.

The present invention discloses how to produce wrought alloys which inherently have high corrosion resistance and do not require cladding but which have strength properties closely approaching those of the best of the heat-treatable wrought alloys of the prior art. The strength properties of the wrought alloys provided according to the present invention and the heat-treatable alloys now in use are even more comparable when the latter are taken as clad alloys, which indeed must be done for a fair comparison in the cases of the many specific uses where corrosion resistance is required. Of course, it follows that the strength properties of alloys provided according to the present invention far exceed those of the commercially useful, non-heat-treatable wrought aluminum alloys of the prior art.

I have discovered that certain aluminum-magnesium compositions, heretofore regarded as casting compositions, will respond under certain conditions to the common mechanical working processes to be converted to wrought alloys having the advantages mentioned above. These alloys comprise what may apparently be most appropriately characterized as non-heat-treatable alloys which may be employed either in the cold worked or annealed state. The surface finishes of these alloys are of exceptionally high quality and they are therefore much superior in this respect even to present commercially useful, non-heat-treatable wrought alloys.

Accordingly, an object of the invention is to provide wrought aluminum alloys which have strength properties comparable with the best heat-treatable wrought aluminum alloys of the prior art, but which do not require cladding for use in numerous applications where such prior art heat-treatable wrought aluminum alloys would require cladding.

2

Another object of the invention is to provide wrought aluminum alloys which are superior to all others in many applications in the manufacture of architectural structural components, marine equipment, cooking utensils, dairy equipment and other uses.

As an embodiment of the invention (which is given by way of example and not by way of limitation to all the precise details thereof) an alloy is provided from those alloys comprising magnesium 5-8%, titanium .10-.25%, manganese .10-.25%, beryllium .0005-.05%, balance, aluminum; or from alloys comprising the same components plus .001-.05% boron, this element appearing to be of benefit in most instances. Other metals which may be present may include copper, iron, silicon and the like, and they can be considered impurities. Impurities should not exceed a combined total of about .50% of the alloy.

Certain alloys included within the ranges specified above have gained wide acceptance throughout the aluminum industry and are presently commonly known as Almag 35. They are, however, used only in the cast condition as produced in sand or permanent molds or the like. In this connection, reference is made to U. S. Patents 2,564,044; 2,583,473 and 2,733,991. These Almag 35 alloys have not been found useful for the manufacture of wrought aluminum alloy products.

The alloy provided from those specified above is soaked for a period of hours at a temperature of from about 700-750° F. The minimum soaking time may vary from 1/4 hour to 40 hours or more, preferably not over 24 hours in most cases, depending on the massiveness of the metal. If any doubt exists as to sufficiency of the soaking of a given kind and shape of charge, the soaking time may be made excessive and may then be varied downwardly in succeeding trials with similar charges until a workable minimum is established.

After soaking, the charge is formed by operations which involve mechanical working such as forging, rolling, extruding, and the like, until the charge is reduced in cross-sectional area about 50% and preferably at least within the range of about from 40 to 60%. During this initial reduction, the metal is maintained at temperatures not exceeding, and not substantially below, the previously mentioned range of from about 700-750° F. This may be done, for example, by frequent passes through or into and out of a furnace pit or other hot zone. After this initial reduction, the metal is fully annealed by repeating the soaking step at the previously mentioned range of from about 700-750° F.

An aluminum-magnesium alloy provided in this manner may be regarded at this stage as a processed raw material which may be further reduced at later times (and after shipment, if desired) by cold working during conventional forming operations at least down to 16% of starting cross-section. It can be thereafter annealed, if desired.

An aluminum-magnesium product made according to the above disclosure was found to have an ultimate strength of 75,000 pounds per square inch, a yield strength of 60,000 pounds per square inch, and an elongation of about 5%. After full annealing, the same material was found to have an ultimate strength of 50,000 pounds per square inch, a yield strength of 26,000 pounds per square inch, and an elongation of 32%.

For comparison purposes, these results are set forth in the following tables together with several of the well-

known wrought aluminum alloys of both the heat-treatable and non-heat-treatable types:

presently known heat-treatable wrought aluminum alloys.

Comparison table—Not annealed

|                                     |                                     |                                                   | Material-Alcoa Alloy Desig. | Ult. Strength, p. s. i. | Yield Strength, p. s. i. | Elong., percent |
|-------------------------------------|-------------------------------------|---------------------------------------------------|-----------------------------|-------------------------|--------------------------|-----------------|
| Present Product, Work-hardened..... |                                     |                                                   | none                        | 75,000                  | 60,000                   | 5               |
| Standard aluminum alloys.           | Non-heat-treatable—Cold worked..... |                                                   | 52S                         | 41,000                  | 36,000                   | 7               |
|                                     | Clad ("Alclad").....                | solution heat treated and then cold worked.       | 56S                         | 58,000                  | 48,000                   | 7               |
|                                     |                                     | solution heat treated and then artificially aged. | 14S                         | 63,000                  | 40,000                   | 20              |
|                                     |                                     | solution heat treated and then cold worked.       | 24S                         | 64,000                  | 44,000                   | 15              |
|                                     |                                     | solution heat treated and then artificially aged. | 14S                         | 68,000                  | 60,000                   | 10              |
|                                     | Heat treatable.....                 |                                                   | 75S                         | 76,000                  | 67,000                   | 11              |
|                                     | Not clad.....                       | solution heat treated and then cold worked.       | 14S                         | unknown                 | unknown                  | —               |
|                                     |                                     | solution heat treated and then artificially aged. | 24S                         | 70,000                  | 50,000                   | 16              |
|                                     |                                     |                                                   | 14S                         | 70,000                  | 60,000                   | 13              |
|                                     |                                     |                                                   | 75S                         | 82,000                  | 72,000                   | 17              |

Comparison table—Annealed

|                                      |                         |  | Material-Alcoa Alloy Desig. | Ult. Strength, p. s. i. | Yield Strength, p. s. i. | Elong., Percent |
|--------------------------------------|-------------------------|--|-----------------------------|-------------------------|--------------------------|-----------------|
| Present Product, Fully annealed..... |                         |  | none                        | 50,000                  | 26,000                   | 32              |
| Standard aluminum alloys.            | Non-heat-treatable..... |  | 52S                         | 27,000                  | 12,000                   | 25              |
|                                      |                         |  | 56S                         | 42,000                  | 22,000                   | 25              |
|                                      | Clad ("Alclad").....    |  | 14S                         | 25,000                  | 10,000                   | 21              |
|                                      |                         |  | 24S                         | 26,000                  | 11,000                   | 19              |
|                                      | Heat treatable.....     |  | 75S                         | unknown                 | unknown                  | —               |
|                                      | Not Clad.....           |  | 14S                         | 27,000                  | 14,000                   | 18              |
|                                      |                         |  | 24S                         | 27,000                  | 11,000                   | 19              |
|                                      |                         |  | 75S                         | 33,000                  | 15,000                   | 17              |

It is believed apparent that specific details of the practice of the invention may be varied without essential departure from the teachings thereof. All such variations are contemplated as may be covered by the following claims, either literally or under the doctrine of equivalents.

What is claimed is:

1. A method for making a wrought aluminum alloy material comprising soaking a body of metal comprising magnesium 5 to 8%, titanium .10 to .25%, manganese .10 to .25%, beryllium .0005 to .05%, impurities not more than .50%, balance aluminum, for a period of from 15 minutes to 40 hours at a temperature of about from 700 to 750° F., reducing said body by forming to about from 40 to 60% of starting cross-section while maintaining said body within a temperature range not greater than and not substantially below about from 700 to 750° F. and then further soaking the body at about from 700 to 750° F. to fully anneal it whereby the resulting alloy material is greatly further reducible by cold working and is capable of achieving thereby strengths comparable with those of presently known heat-treatable wrought aluminum alloys while also having corrosion resistance far superior to that of presently known heat-treatable wrought aluminum alloys.

2. A method for making a wrought aluminum alloy material comprising soaking a body of metal comprising magnesium 5 to 8%, titanium .10 to .25%, manganese .10 to .25%, boron .001 to .05%, beryllium .0005 to .05%, impurities not more than .50%, balance aluminum, for a period of from 15 minutes to 40 hours at a temperature of about from 700 to 750° F., reducing said body by forming to about from 40 to 60% of starting cross-section while maintaining said body within a temperature range not greater than and not substantially below about from 700 to 750° F. and then further soaking the body at about from 700 to 750° F. to fully anneal it whereby the resulting alloy material is greatly further reducible by cold working and is capable of achieving thereby strengths comparable with those of presently known heat-treatable wrought aluminum alloys while also having corrosion resistance far superior to that of

3. A method for making a wrought aluminum alloy material comprising soaking a body of metal comprising magnesium 5 to 8%, titanium .10 to .25%, manganese .10 to .25%, beryllium .0005 to .05%, impurities not more than .50%, balance aluminum, for a period of from 15 minutes to 40 hours at a temperature of about from 700 to 750° F., reducing said body by forming to about from 40 to 60% of starting cross-section while maintaining said body within a temperature range not greater than and not substantially below about from 700 to 750° F., then further soaking the body at about from 700 to 750° F. to fully anneal it, then further reducing the resulting alloy material by cold working at least down to 16% of starting cross-section, and then fully annealing the alloy material as so reduced whereby the resulting fully annealed material has strengths favorably comparable with those of presently known fully annealed wrought aluminum alloys.

4. A method for making a wrought aluminum alloy material comprising soaking a body of metal comprising magnesium 5 to 8%, titanium .10 to .25%, manganese .10 to .25%, boron .001 to .05%, beryllium .0005 to .05%, impurities not more than .50%, balance aluminum, for a period of from 15 minutes to 40 hours at a temperature of about from 700 to 750° F., reducing said body by forming to about from 40 to 60% of starting cross-section while maintaining said body within a temperature range not greater than and not substantially below about from 700 to 750° F., then further soaking the body at about from 700 to 750° F. to fully anneal it, then further reducing the resulting alloy material by cold working at least down to 16% of starting cross-section, and then fully annealing the alloy material as so reduced whereby the resulting fully annealed material has strengths favorably comparable with those of presently known fully annealed wrought aluminum alloys.

5. A wrought aluminum alloy material comprising a body of metal comprising magnesium 5 to 8%, titanium .10 to .25%, manganese .10 to .25%, beryllium .0005 to .05%, impurities not more than .50%, balance aluminum, said body being in a state resulting from soaking

for a period of hours at about from 700 to 750° F., and then reduction by forming to about from 40 to 60% of starting cross-section while being maintained within a temperature range not greater than and not substantially below about from 700 to 750° F., and finally full annealing at about from 700 to 750° F., said body being characterized by being further reducible by cold working at least down to 16% of starting cross-section whereupon its ultimate tensile strength is in the vicinity of 75,000 pounds per square inch and its yield strength is in the vicinity of 60,000 pounds per square inch.

6. A wrought aluminum alloy material comprising a body of metal comprising magnesium 5 to 8%, titanium .10 to .25%, manganese .10 to .25%, boron .001 to .05%, beryllium .0005 to .05%, impurities not more than .50%, balance aluminum, said body being in a state resulting from soaking for a period of hours at about from 700 to 750° F., and then reduction by forming to about from 40 to 60% of starting cross-section while being maintained within a temperature range not greater than and not substantially below about from 700 to 750° F., and finally full annealing at about from 700 to 750° F., said body being characterized by being further reducible by cold working at least down to 16% of starting cross-section whereupon its ultimate tensile strength is in the vicinity of 75,000 pounds per square inch and its yield strength is in the vicinity of 60,000 pounds per square inch.

7. A wrought aluminum alloy material comprising a body of metal comprising magnesium 5 to 8%, titanium .10 to .25%, manganese .10 to .25%, beryllium .0005 to .05%, impurities not more than .50%, balance aluminum, said body being in a state resulting from soaking for a period of hours at about from 700 to 750° F., and then

reduction by forming to about from 40 to 60% of starting cross-section while being maintained within a temperature range not greater than and not substantially below about from 700 to 750° F., then full annealing at about from 700 to 750° F., then further reduction by cold working at least down to 16% of starting cross-section, and then full annealing at about from 700 to 750° F., said body being characterized by an ultimate tensile strength in the vicinity of 50,000 pounds per square inch and a yield strength in the vicinity of 26,000 pounds per square inch.

5 8. A wrought aluminum alloy material comprising a body of metal comprising magnesium 5 to 8%, titanium .10 to .25%, manganese .10 to .25%, boron .001 to .05%, beryllium .0005 to .05%, impurities not more than .50%, balance aluminum, said body being in a state resulting from soaking for a period of hours at about from 700 to 750° F., and then reduction by forming to about from 40 to 60% of starting cross-section while being maintained within a temperature range not greater than and not substantially below about from 700 to 750° F., then full annealing at about from 700 to 750° F., then further reduction by cold working at least down to 16% of starting cross-section, and then full annealing at about from 700 to 750° F., said body being characterized by an ultimate tensile strength in the vicinity of 50,000 pounds per square inch and a yield strength in the vicinity of 26,000 pounds per square inch.

10 20 25 30 35

References Cited in the file of this patent  
Transactions of the A. S. M., vol. 44, 1952. (Pages 336 through 347, page 338 especially relied upon.)

UNITED STATES PATENT OFFICE  
CERTIFICATE OF CORRECTION

Patent No. 2,841,512

July 1, 1958

Hugh S. Cooper

It is hereby certified that error appears in the printed specification of the above numbered patent requiring correction and that the said Letter Patent should read as corrected below.

Column 3, line 61, and column 4, lines 35 and 54, for "25%", each occurrence, read --.25%--.

Signed and sealed this 7th day of October 1958.

(SEAL)

Attest:

KARL H. AXLINE

Attesting Officer

ROBERT C. WATSON  
Commissioner of Patents